

## UNITED STATES PATENT OFFICE

HARRY HINTZE, OF PATERSON, NEW JERSEY

## PROCESS FOR WEIGHTING OF NATURAL AND ARTIFICIAL SILK FIBERS

No Drawing.

Application filed May 18, 1932. Serial No. 611,244.

In processes heretofore made use of for weighting of natural silk and other fibers, in the form of skeins and woven or knitted fabrics, a number of chemical substances 5 were brought into contact with the fibers.

In practice the use of metallic compounds such as iron—for black and navy blue only—zinc, alumina, bismuth, tin and lead has been resorted to; however, a tin-metal solution has 10 proven best.

According to the well-known methods now and heretofore employed, as for instance, the natural, boiled-off silk is treated first with a solution of tetra-chloride of tin— $\text{SnCl}_4$ , of 15 about 22° Baumé strength at a temperature of 60° F. for some time, and then is rinsed thoroughly with hard water—6°—9° hardness—in order to hydrolyze the tin and to precipitate the same on the fiber in the form of 20 stannic acid— $\text{H}_2\text{SnO}_4$ . This stannic acid precipitate is then fixed by a treatment of the silk with di-sodium phosphate— $\text{Na}_2\text{PO}_4$ , of about 7° Baumé strength at about 60° C. 25 and thereafter rinsed in soft water. The stannic chloride baths and the phosphate baths are alternately repeated until the desired degree of weighting has been obtained, and after each bath or treatment, the silk 30 has to undergo a water rinsing or neutralization as described above. After the last phosphate bath and subsequent rinsing, a treatment in a solution of sodium silicate— $\text{Na}_2\text{SiO}_4$ —of about 1° Baumé strength and 35 at a temperature of 45° C. is applied. The silk which has been manipulated in this manner and weighted with complex compounds of tin, phosphate and silicate, is then rinsed, soaped and scoured and is ready to be further 40 processed by dyeing and finishing.

The operations described in the foregoing paragraph as well as other methods of weighting with various substances, are well known and generally practiced in the industry at the present time.

45 On account of the tendering effect on the tensile strength of the fiber of too heavy and too many charges of tin-phosphate compounds, and their costs, and the time necessary for the many washings, the weighting process with tin is generally limited to four

applications of tin-phosphate and their attendant rinsings, with an average increase in weight of about 11% for each passage and aggregate gain of about 40% over the weight of the boiled-off silk. 55

The purpose of the present invention is to improve upon the methods now in use and to provide a process which will yield very considerably more weight with the same number of passes or one additional pass and which 60 at the same time imparts desirable qualities to the natural silk and other synthetic fibers.

In the course of extensive experiments, it was found that natural silk and other synthetic fibers charged with metals such as iron, alumina, zinc and tin show a marked affinity for plumbic chloride or di-chloride of lead— $\text{PbCl}_2$ . This particular lead compound resembles in chemical structure the well-known pink salt— $\text{SnCl}_2$ —of commerce and the tetra-chloride of tin— $\text{SnCl}_4$ —now universally used 65 for weighting purposes. On account of the even and level results obtainable in weighting with di-chloride of lead and its pure white color, it is far superior to other lead compounds, but especially to acetate of lead— $\text{Pb}(\text{C}_2\text{H}_2\text{O}_2)_2$ —which has been used for 70 weighting purposes. 75

Di-chloride of lead, while known to chemical science, has up to the present time never 80 been commercially produced to any extent, has not been offered for sale by leading manufacturers, nor is its price quoted, and has therefore been unobtainable as an article of commerce and has never been used in the art 85 of weighting natural silk and synthetic fibers, known as artificial silk.

For purposes of illustration the silk weighting process is cited: In the present 90 invention the natural, boiled-off silk is treated two, three or four times in the old and well-known manner with stannic metals and sodium phosphate and thorough rinsings after each bath, producing a gain of from 95 20%—45% over the weight of the boiled-off silk. The silk is then worked for one half hour in a bath containing about 5% of monochlor-acetic acid or formic acid—based on the weight of the raw good—at 150° F. and subsequently in a bath of an aqueous sus- 100

sension of di-chloride of lead of 1°-5° Baumé strength at a temperature of about 160° F. for one hour. After this treatment the goods are copiously rinsed in hard 5 water—6°-9° hardness—in order to hydrolyze the lead compound and to precipitate same on the fiber in the form of plumbic hydroxide,  $Pb(OH)_2$ . This plumbic hydroxide precipitate is then fixed on the fiber by 10 a treatment in an aqueous solution of ammonia carbonate— $NH_4H.CO_3$ —of about 3°-6° Baumé strength and of a temperature of 60° F. for about one hour. Subsequently 15 the goods are thoroughly rinsed in soft water and are then ready for silicating and soaping and can be further processed in the usual way by dyeing and finishing.

In order to facilitate the holding in suspension of the di-chloride of lead, it is recommended to add a deci-normal solution of 20 sodium thiosulphate to the bath.

The silicating operation can also be carried out immediately after the tin-phosphate treatment instead of after the lead-weighting step. 25

The fibroin of the silk forms a homogenous compound of a very complex nature with the plumbic hydroxide carbonate of ammonia and the stannic acid-phosphate previously 30 deposited in the interior of the fiber by the tin-phosphate treatment.

It is also possible to use instead of carbonate of ammonia for the fixing of the plumbic hydroxide on the fiber, hydroxide 35 of ammonia, mono-sodium phosphate, di-sodium phosphate or tri-sodium phosphate.

Continuing with the example, if the tin-weighted silk is treated in a bath of proper proportions and temperatures according to 40 the directions given above, the tin-weighted natural silk and synthetic fibers are heavily charged with lead-metal compounds and it is possible to obtain from 25% to 65% gain in weight by one single immersion in a di-chloride of lead suspension over and above and 45 in addition to that of the tin-weighted goods.

Added advantages of the process covered by this application are the facts that silk materials so treated show very considerable 50 more tensile strength than those merely tin-weighted. Indeed, tin-weighted natural silk as well as synthetic fibers, tendered in the tin-weighted process, so-called "tender goods" can be restored to their normal strength and 55 have it materially improved by an application of the di-chloride-carbonate of ammonia treatment.

The white produced with this method of weighting is of pure white quality and the 60 goods, therefore, do not have to be bleached for this particular shade nor for other tints requiring a pure white ground, as is the case with goods treated with other forms of lead compounds such as acetate of lead.

65 Goods intended for printing purposes lend

themselves to discharge work under certain conditions.

Furthermore, a decided advantage, compared to only tin-weighted natural silk and synthetic fibers, is the diminished shrinkage 70 of di-chloride of lead-treated goods, representing a gain of from three to six percent in yardage. The draping qualities of silk treated by the methods of this application are far superior, furnishing a fuller and more "mellow hand" and requiring less finishing materials, without, however, impairing the desirable and peculiar qualities of silk. 75

The result of the process described above is 80 a composite fiber consisting in a minor part of the fibroin of the silk and in a major part of the compound of tin, lead, phosphate and ammonia carbonate, homogeneously combined and which will give off none of its component elements when treated with acetic acid 85 or other liquids with which the natural silk and synthetic fibers, known as artificial silk, may come in contact during dyeing and finishing operations or when being worn and exposed to perspiration and other secretions 90 of the human body.

It is understood that the term "bath" employed in the specification and claims designates an "aqueous bath". The term "fiber" 95 in the specification and claims is used in a generic sense and signifies natural or artificial silk fibers in the form of skeins, knitted fabric, woven fabric or any material the body of which is formed of fibers.

I claim:

1. The process of weighting natural and 100 artificial silk fiber which comprises treating said fiber in separate baths with tin-weighting and fixing agents, treating said fiber in a bath containing di-chloride of lead, and subsequently treating said fiber in a fixing bath.

2. A step in the process of weighting natural and artificial silk fiber which comprises the treatment of the fiber in a bath containing lead chloride. 110

3. The process of weighting natural and 115 artificial silk fiber which comprises treating said fiber in separate baths with tin-weighting and fixing agents, treating said fiber in a bath containing di-chloride of lead and subsequently treating said fiber in a bath containing ammonium carbonate.

4. The process of weighting natural and 120 artificial silk fiber which comprises treating said fiber in separate baths with tin-weighting and fixing agents, treating said fiber in a bath containing di-chloride of lead and subsequently treating said fiber in a bath containing ammonium hydroxide.

5. The process of weighting natural and 125 artificial silk fiber which comprises treating said fiber in separate baths with tin-weighting and fixing agents, treating said fiber in a bath containing di-chloride of lead and subsequently treating said fiber in a bath con- 130

taining at least one material selected from a group consisting of mono-sodium phosphate, di-sodium phosphate and tri-sodium phosphate.

5 6. A step in the process of weighting natural and artificial silk fiber which comprises the treatment of the fiber in a bath containing di-chloride of lead and a salt inducing the solubility of lead di-chloride in  
10 water.

7. A step in the process of weighting natural and artificial silk fiber which comprises the treatment of the fiber in a bath containing di-chloride of lead and sodium  
15 thiosulphate.

8. The process of weighting natural and artificial silk which comprises treating said fiber in separate baths with tin-weighting and fixing agents, treating said fiber in a  
20 bath containing sodium silicate, treating said fiber in a bath containing di-chloride of lead, and subsequently treating said fiber in a fixing bath.

9. The process of weighting natural and  
25 artificial silk fiber which comprises treating said fiber in separate baths with tin-weighting and fixing agents, treating said fiber in a bath containing di-chloride of lead, treating said fiber in a fixing bath, and finally  
30 treating said fiber in a bath of sodium silicate.

10. The process of weighting natural and artificial silk fiber which comprises treating said fiber in a bath containing lead chloride and subsequently treating said fiber in a fix-  
35 ing bath.

HARRY HINTZE.

40

45

50

55

60

65